

## UNITED STATES PATENT OFFICE

2,113,034

## STARCH SIZING OF PAPER

Ben W. Rowland, Appleton, Wis., and Jordan V. Bauer, Chicago, Ill., assignors to Stein, Hall Mfg. Co., Chicago, Ill., a corporation of Delaware

No Drawing. Application June 5, 1935,  
Serial No. 25,124

5 Claims. (Cl. 92—21)

The invention relates to the precipitation of starch upon fibers used in the manufacture of paper. It is of particular value in connection with the use of starch in the furnish.

5 The word "starch" as used herein, is intended to include not only the various kinds of starch proper, such as corn starch, potato starch, tapioca starch, etc., or flours containing said starches, but also degradation products such as 10 so-called modified starches, oxidized starches, starch gums, etc.

The advantage due to the use of starch in the manufacture of paper has long been recognized. Starch in various ways has been employed in 15 the coating or finishing of the paper web after the formation of the latter on the wire. Various proposals have also been put forward for incorporating starch in the furnish, before formation of the web, but it has been found that 20 where a considerable quantity of starch is supplied to the furnish, only a relatively small amount of such starch is found in the formed web. This apparently is due to the fact that starch, being a dispersible colloid, is not precipitated upon or retained by the fibers in 25 any large amount and, therefore, to a large extent, is retained by, and is carried off with, the white water which drains out of the web. As a result, it has not been possible by ordinary methods to incorporate starch with the web in an amount exceeding a few per cent of the weight of fiber on the dry basis. Also, in order to secure the retention of such relatively small percentage of starch, it has been necessary to use in 30 the furnish a much greater percentage, thereby causing such waste and expense that, practically speaking, the use of starch heretofore in the furnish has been attended with no substantial commercial advantage.

40 In the co-pending application of one of us, Rowland, Serial No. 726,125, filed May 17, 1934, it is proposed to utilize for sizing a colloidally dispersed starch which is precipitated on the fiber by the addition of a precipitant after the stock has been completely worked in the beater and Jordan and after the colloidal starch has been thoroughly disseminated in the stock. That procedure has been quite satisfactory and 45 efficient.

50 It is very desirable, however, for practical reasons, that the starch be added to the beater, rather than between the Jordan engine and the paper-making machine. If added to the beater, the size may be run in with a minimum of in-

convenience and with substantially no modification of the standard paper plant setup.

We have found that when ordinary starches are added dry and uncooked to the beater, they are too tough to be broken up by the Jordan, 5 whereas if they are cooked to any appreciable extent they are too soft and are dispersed by the Jordan beyond the limits of possible precipitation and, therefore, are ineffective as sizing agents if introduced into the process at this 10 point.

After extensive investigation, we have discovered that especially treated starches which are considerably tougher than ordinary or "natural" starches function perfectly as sizes 15 when introduced into the beater. The beating operation, instead of destroying or reducing the value of said starches as in the case of ordinary starches, seems to condition them and place them in such a state of dispersion as to produce their 20 optimum sizing effect.

In accordance with our special starch treatment, the starch granules are toughened to the extent that they will not be as readily dispersed when they are gelatinized or swollen, for example, by means of boiling water or caustic solution, as ordinary boiled starch. Our special starch treatment may be carried out to the extent that the starch granules will be so toughened that they will not swell or gelatinize in 30 water even when subjected to prolonged boiling temperatures, or such treatment may be carried only to the extent that a slight toughening of the starch granules will be effected, in which latter case the starch granules can be dispersed 35 by means of hot water or caustic solution, but to a substantially lesser degree than untreated starch.

Starch treated in accordance with our invention, when cooked in water and alkali will form a 40 suspension of swollen starch granules which can be readily precipitated by the addition of sufficient acid or acid salt to reduce the pH to about 5 or less. Such precipitated starch can again be brought into a state of suspension by the addition of a sufficient amount of alkali to bring the aqueous medium to a pH of about 10 or above.

*Example*

The furnish may consist of soda pulp or sulfite pulp, or rag stock, or a combination of the same, and may include also a substantial percentage of ground wood if a relatively cheap paper is being produced. A suitable percentage of mineral filler may also be included in the 55

furnish. In fact, the invention appears to work well with almost any kind of furnish used in the manufacture of paper.

The special starch utilized in our invention 5 may be prepared in the following manner:

1,260 pounds of powdered corn or other raw starch is placed in a steam jacketed mixer, preferably equipped with a power-driven agitator. While the starch is being agitated a mixture of 10 2,600 cc. of 40 per cent formaldehyde solution, 1,500 cc. of 56 per cent acetic acid, and 4,500 cc. of water are sprayed in and the total mass is mixed for about a half hour, or until the liquid ingredients have been thoroughly incorporated 15 with the starch. At the end of this time, steam at about 50 pounds' pressure is turned into the jacket of the mixer and the material is heated for a period of one to two hours or until control tests show the desired degree of action on the 20 starch has taken place. The starch is then dumped out of the mixer and allowed to cool, after which it is ready for use.

A somewhat different method of treating the starch which gives the same desirable results is 25 as follows:—

1,000 pounds of starch is mixed with 1,200 pounds of water in a suitable tank equipped with an agitator. To this mixture is added 10,000 cc. of 40 per cent formaldehyde and 2,000 cc. of 18° 30 Bé. hydrochloric acid, and the mass is held at a temperature of about 75° F. and agitated for about 24 hours, or until control tests show that the desired degree of action on the starch has taken place. At the end of this time, the water 35 is separated from the starch by means of a filter or a centrifuge and the starch is washed several times with clean water. It is then dried by means of a starch-drying kiln or a vacuum-type dryer. It is then ready for use.

40 The control tests referred to above are such as will show that the starch, after the above treatment, will swell in hot water or in a caustic solution to form a suspension or gel but will be reprecipitated by acid. The following comparative 45 tests will illustrate certain properties of our special starch as compared with ordinary starch.

Ten grams each of ordinary corn starch and our 45 treated corn starch are cooked up separately with 150 cc. of water and .01 grams of caustic soda 50 to a temperature of 195° F. and held at this temperature for 15 minutes. A 20-gram portion is taken from each of these cooked samples of gelatinized starch and dispersed in 210 cc. of distilled water. The subsequent starch suspensions are 55 poured into 250 cc. graduates and placed side by side. The pH of these dispersed starches will be about 12.0. To each of the graduates is then added 6 cc. of 1/10 N. sulphuric acid and distributed by shaking in the graduate. Immediately 60 after the acid is added to the dispersion of the treated starch a flocculent precipitate of starch forms and begins to settle out; whereas in the case of the ordinary corn starch dispersion there is no noticeable precipitation. The pH of 65 the starch dispersion after the addition of the acid is approximately 3.0.

It should be understood that the above methods 70 are merely specific examples of how we treat the starch to obtain the desired degree of modification and that we do not wish to limit ourselves to these specific examples of treatment. The acid ingredient used in the above examples is merely a catalyst and as such accelerates the reaction between the formaldehyde and the starch 75 and enables the use of smaller amounts of form-

aldehyde than would otherwise be practical, it is not necessary, however, for the success of the process. For the first method of treatment just described practically any volatile acid may be used as a catalyst but we prefer to use acetic acid because it has less tendency to dextrinize starch than such acids as hydrochloric or nitric. In the second method of treatment practically any water soluble acid can be used as the catalyst.

Our special starch is prepared for use as follows: A suitable quantity of water corresponding to 15 times the weight of the starch is warmed to a temperature of between 56° and 60° C. The dry starch is then put into the water and stirred 15 until the lumps are thoroughly wetted out. A quantity of alkali such as sodium hydroxide in any concentration, preferably around 20 per cent in water and amounting to 7.3 pounds of dry caustic per 100 pounds of starch being treated, 20 is introduced into the starch mixture with stirring. As soon as it has been thoroughly stirred in, the agitation may be discontinued and the batch allowed to stand for from 10 to 15 minutes, during which interval the starch swells into a 25 gelatinous condition and becomes quite thick and at first white and opaque, but in a few minutes transparent and glassy. It is then ready for addition to the beater. This condition of alkalinity in the starch solution will generally render the 30 beater contents appreciably alkaline. Rosin size may be introduced, as well as other ingredients of the furnish, toward the end of the beating cycle to prevent foaming, although our mill experience with this procedure has not as yet presented a foaming problem. Alum, which is the 35 remaining addition to effect precipitation of the starch and also of the rosin size, is withheld until the furnish has passed through the Jordan and there it may be added to bring the furnish 40 acidity down to any pH preferred by the mill, which is usually a pH necessary for effective rosin sizing. We have added the alum at different points at different mills, and find that it is immaterial at what point we add it so long as it 45 is thoroughly mixed in.

While in our preferred practice the alum is introduced between the Jordan and the paper machine, satisfactory results may be obtained if the alum is added to the beater immediately following the introduction of the starch and rosin. Since, when starches of the special type herein considered are used, precipitation will not occur until after the furnish has passed through the Jordan and the starch has become broken down, 55 in case the alumina has previously been formed in the beater, it would be immediately available to effect precipitation at the moment the starch is broken down in the Jordan.

The furnish prepared as described above is 60 run through the paper machine in the ordinary manner without any material change in the machine practice.

Paper made according to the process described above has many advantages over paper not containing starch and also over paper which contains the same amount of ordinary starch incorporated in the same grade of paper according to the old practice, such as greatly increased strength.

Various modifications and variations coming 70 within the spirit of our invention will doubtless suggest themselves to those skilled in the art. Hence, we do not wish to be limited to the specific embodiments and details herein disclosed except to the extent indicated by the appended claims, 75

which are to be interpreted as broadly as the state of the art will permit.

We claim as our invention:

- 5 1. The improvement in the art of paper-making, which comprises introducing into the furnish before the completion of the beating operation an alkaline dispersion of a tough, formaldehyde treated raw starch which is capable of being colloidally dispersed by the beating action and will 10 retain after such beating its ability to be precipitated on the fiber, and, prior to the paper-forming operation, adding alum to the furnish so as to precipitate said starch upon the fiber in finely-divided form.
- 15 2. The improvement in the art of paper making, which comprises introducing into the furnish, before the completion of the beating operation, an alkaline dispersion of a tough starch produced by treating a raw starch with formaldehyde and, 20 prior to the paper-making operation, adding sufficient acidic material to the furnish to precipitate said starch upon the fiber in finely-divided form.
- 25 3. The improvement in the art of paper making, which comprises introducing into the furnish, before the completion of the beating operation, an alkaline dispersion of a tough starch produced

by treating a raw starch with formaldehyde and an acid catalyst and, prior to the paper-making operation, adding sufficient alum to the furnish to precipitate said starch upon the fiber in finely-divided form.

5 4. The improvement in the art of paper-making, which comprises introducing into the furnish before the completion of the beating operation an alkaline dispersion of a tough, formaldehyde treated raw starch which is capable of being colloidally dispersed by the beating action and will 10 retain after such beating its ability to be precipitated on the fiber, and precipitating said starch upon the fiber by the addition of acidic material.

15 5. The improvement in the art of paper-making, which comprises introducing into the furnish, before the completion of the beating operation, an alkaline dispersion of a tough starch produced by treating a raw starch with formaldehyde and an acid catalyst and, prior to the paper-making 20 operation, adding sufficient acidic material to the furnish to precipitate said starch upon the fiber in finely divided form.

BEN W. ROWLAND.  
JORDAN V. BAUER. 25